

# UNITED STATES PATENT OFFICE.

ERNST OTTO GRÜNERT, OF MEISSEN, SAXONY, GERMANY.

## MANUFACTURE OF LINOPHANIES OR TRANSLUCENT PICTURES.

SPECIFICATION forming part of Letters Patent No. 314,931, dated March 31, 1885.

Application filed December 3, 1884. (No specimens.)

*To all whom it may concern:*

Be it known that I, ERNST OTTO GRÜNERT, of Meissen, in the Kingdom of Saxony and German Empire, have invented certain Improvements in the Manufacture of Linophanies or Translucent Pictures, Ornaments, &c., from Paper-Pulp, of which the following is a specification.

My new method of making "linophanies," so called, comprises the following steps: Paper-pulp, white or colored, in a liquid or semi-liquid state, is poured into a mold, usually of metal, the bottom of which is engraved to form or produce the desired design or picture. Enough pulp must be poured in to leave a thin film of paper over the highest lines of the engraved surface, when the pulp is dried, as will be hereinafter described. I may here remark that those portions of the engraving which correspond to the dark portions or shades of the picture are cut deeper than those which correspond to the lights of the picture, the depth varying with the depth of the shade. Upon the paper-pulp in the mold I spread a piece of gauze, fine linen, or other similar material that will not adhere to the pulp, but will permit the passage of water, and on this I place blotting-paper in one or more layers, and then subject the whole to pressure in any ordinary press. The blotting-paper is thus caused to absorb the greater portion of the water from the pulp, and the latter is pressed into all the finer lines of the engraving and suitably compacted. For the blotting-paper I may substitute any other similar absorbent material—as some kinds of felt, for example. After removing the mold from the press I remove the blotting-paper and the linen or gauze separating material, and then, by preference, subject the mold containing the partially-dried pulp to artificial heat, as in a stove or kiln, to dry out the remaining moisture. The dried paper-pulp is now removed from the mold, and will be found to consist of a continuous imperforated paper leaf bearing the design or picture, which will be fully brought out when the sheet is held up between the eye and a strong light. The thinner portions of the sheet will represent the lights of the picture, and the thicker

(and less translucent) portions will represent the shades.

The picture or ornament thus produced is called a "linophany," and may be employed for lamp or gas shades, and for transparent pictures for windows, &c., or, indeed, for any ornamental purposes to which such a picture or design is adapted.

In lieu of using artificial heat to dry the pulp in the mold, I may allow it to dry by the natural evaporation of its moisture; but I prefer to employ a heated kiln.

The mold is usually engraved, but the design may be formed in any way—as by pressure from a hardened relief-plate, for example.

Having thus described my invention, I claim—

1. The herein-described method of manufacturing "linophanies," so called, which consists in, first, pouring paper-pulp into a properly-prepared mold, as described; second, covering said pulp with a previous sheet of gauze or its specified equivalent, and then placing upon said sheet blotting-paper or other similar absorbent material; third, subjecting the contents of the mold to pressure, and, fourth, removing the absorbent material and the gauze, in order that the pulp may dry in the mold, substantially as described.

2. The herein-described method of manufacturing "linophanies," so called, which consists in, first, pouring paper-pulp into a properly-prepared mold, as described; second, covering said pulp with a previous sheet of gauze or its specified equivalent, and then placing upon said sheet blotting-paper or other similar absorbent material; third, subjecting the contents of the mold to pressure, and, fourth, removing the absorbent material and the gauze, and, fifth, subjecting the mold and the pulp contained therein to artificial heat, in order to complete the drying of the pulp in the mold, substantially as described.

This specification signed by me this 24th day of October, 1884.

ERNST OTTO GRÜNERT.

Witnesses:

CARL T. BURKHARDT,  
B. ROI.